



US005380482A

**United States Patent** [19]

Maginnis et al.

[11] **Patent Number:** 5,380,482[45] **Date of Patent:** Jan. 10, 1995

- [54] **METHOD OF MANUFACTURING INGOTS FOR USE IN MAKING OBJECTS HAVING HIGH HEAT, THERMAL SHOCK, CORROSION AND WEAR RESISTANCE**
- [75] Inventors: **David B. Maginnis**, Norman; **Frank Maginnis**, Moore, both of Okla.
- [73] Assignee: **Aspen Research, Inc.**, Moore, Okla.
- [21] Appl. No.: 43,628
- [22] Filed: Apr. 2, 1993

**Related U.S. Application Data**

- [63] Continuation-in-part of Ser. No. 780,703, Oct. 18, 1991, abandoned.
- [51] Int. Cl.<sup>6</sup> ..... B22F 3/14; B22F 1/00
- [52] U.S. Cl. ..... 419/33, 419/48; 419/52; 419/44; 419/47; 419/57; 75/255; 75/252; 75/253
- [58] **Field of Search** ..... 419/32, 38, 39, 48, 419/57, 20, 25, 12, 33, 52, 44, 47; 75/235, 244, 249, 254, 255, 252

[56] **References Cited****U.S. PATENT DOCUMENTS**

- 2,915,801 12/1959 Harry ..... 75/27  
 3,248,215 4/1966 Bonis et al. ..... 75/226  
 3,311,522 3/1967 Ladd et al. ..... 156/206  
 3,413,392 11/1968 Meadows ..... 264/102  
 3,591,362 7/1971 Benjamin ..... 419/244  
 3,660,049 5/1972 Benjamin ..... 29/182.5  
 4,325,734 4/1982 Burrage et al. ..... 75/225

- 4,612,165 9/1986 Liu et al. ..... 420/459  
 4,711,761 12/1987 Liu et al. ..... 420/459  
 4,722,828 2/1988 Liu ..... 420/455  
 4,731,221 3/1988 Liu ..... 420/445  
 4,747,990 5/1988 Gauvens et al. ..... 264/322  
 4,801,415 1/1989 Hughes ..... 264/120  
 4,894,086 1/1990 Huether et al. ..... 75/0.5 A  
 4,909,842 3/1990 Dunmead et al. ..... 75/236  
 4,911,762 3/1990 Steinemann ..... 148/2  
 4,946,643 8/1990 Dunmead et al. ..... 419/12  
 4,961,903 10/1990 McKamey et al. ..... 420/79  
 5,098,469 3/1992 Rezhets ..... 75/249

**Primary Examiner**—Donald P. Walsh**Attorney, Agent, or Firm**—Watson, Cole, Grindle & Watson

[57]

**ABSTRACT**

A method of manufacturing ingots for use in making objects having heat, thermal shock, corrosion and wear resistance by formulating a composition of about 17-80% TiB<sub>2</sub> powder, about 0.0 to 4.0% Y<sub>2</sub>O<sub>3</sub> powder, and the balance of NiAl powder, the powders being thoroughly admixed, and placing the admixture into a mold in which it is subjected to a pressure of about 7000 psi and a temperature of about 1400° C. for 20 to 140 minutes in an inert atmosphere, after which the mold is cooled and the ingot is removed and ready for use in manufacturing an object. In some applications the use of a ceramic filler material mixed with the powder is employed to improve the physical characteristics of the finished ingot.

22 Claims, 1 Drawing Sheet





Fig. 4



Fig. 3



Fig. 1



Fig. 2

**METHOD OF MANUFACTURING INGOTS FOR  
USE IN MAKING OBJECTS HAVING HIGH HEAT,  
THERMAL SHOCK, CORROSION AND WEAR  
RESISTANCE**

**CROSS REFERENCE TO RELATED  
APPLICATIONS**

This is a continuation-in-part of application Ser. No. 07/780,703 filed Oct. 18, 1991, now abandoned.

**BACKGROUND OF THE DISCLOSURE**

This invention relates to a composition for use in manufacturing ingots from which parts can be made having heat, thermal shock, corrosion and wear resistance. The method and composition herein is particularly used in manufacturing plungers for use in the glass container manufacturing industry.

Because of thermal shock, wear, and scratches due to particulate contamination in molten glass, there is an increased interest in development of strong, heat resistant, thermal shock, corrosion, and wear resistant material for use in manufacturing plungers as substitutes for cobalt, nickel cast alloys and stainless steel parts presently used in the glass industry. It has been discovered that nickel aluminide, NiAl, composites have good applicability for this purpose because of their high melting temperatures, hardness, and corrosion resistance.

Nickel aluminide has many different stoichiometric compounds. These compounds have significantly different properties. Ni<sub>3</sub>Al with small amounts of boron, or hafnium, or zirconium is disclosed in U.S. Pat. No. 4,612,165. The material was investigated for the U.S. Department of Energy as a substitute for stainless steel. It can be cast into ingots, cold rolled and fabricated into many shapes.

The nickel aluminide used in this disclosure, that is, NiAl, has a much higher melting temperature and is harder than Ni<sub>3</sub>Al but it cannot be cast and still retain its stoichiometric compound. When it is cast the nickel aluminide undergoes a phase separation into nickel and aluminum. This effect can be recognized when studying the phase diagrams in Vol. 8, pp. 262, Eighth Edition of "The American Society For Metals, Metal Handbook". When phase separation takes place the alloy's melting temperature drops significantly and it loses some of its corrosion resistances.

Although several alloy compounds of nickel aluminide exist, NiAl has the favorable characteristic of a high melting temperature, that is, 1640° C. It has been discovered that a composite formed of NiAl and titanium diboride has unexpected levels of hardness and decreased wear rates. The composite formed of NiAl and TiB<sub>2</sub> is characterized by its high temperature properties, high hardness and its lack of depressing the melting point of NiAl.

The NiAl composites of this disclosure are excellent engineering materials and it is expected that they will find many other uses in fabrication of components for turbines, pumps, wear seals, wear plates, foundry tools and other equipment or tools that are exposed to severe wear, thermal shock, and/or high temperatures. The addition of certain platelets, ceramic whiskers or fibers serve to increase the high temperature strength.

For information relating to other compositions having characteristics of hardness of high temperatures and thermal shock and corrosion resistance, see the following U.S. Pat. Nos. 2,915,801; 3,248,215; 3,311,522;

3,413,392; 4,325,734; 4,382,053; 4,612,165; 4,711,761; 4,722,828; 4,731,221, 4,747,990; 4,801,415 and 4,961,903.

**SUMMARY OF THE INVENTION**

5 A method of manufacturing ingots for use in making objects having heat, thermal shock, corrosion and wear resistance is accomplished by providing the materials and the process of forming ingots having these characteristics, the ingots being thereby useable for manufacturing parts. A composition is formed for use in forming ingots of this type, the composition containing about 17 to 80% TiB<sub>2</sub> powder, 0.0 to 4.0% Y<sub>2</sub>O<sub>3</sub> powder and the balance of NiAl powder. The powders being thoroughly admixed. In the preparation of the composition the powders are preferably admixed in a ball mill for a long period, that is, for about 10 to 48 hours to reduce the powder size to a very fine grain.

20 The composition can be improved for certain applications, particularly wherein thermal and physical shock are important, by the incorporation of ceramic reinforcing components in the form of particulate, platelets, fibers or whiskers made of TiB<sub>2</sub>, Al<sub>2</sub>O<sub>3</sub>, B<sub>4</sub>C, TiC, and SiC and mixtures thereof.

25 In another embodiment of the present invention, CrB<sub>2</sub> powder is admixed with NiAl powder to form a composition for use in making ingots. The addition of CrB<sub>2</sub> to the aforementioned mixture of TiB<sub>2</sub> and NiAl also provides a composition which can be used to form an ingot having excellent thermal shock properties and which resists reaction with molten glass at 2100° F.

30 The method of manufacturing an ingot includes milling the powder as above stated and placing the composition in a mold. The powder in the mold is then subjected to high pressure and temperature for a time to cause the admixture to fuse into a high density ingot. It has been learned that the desired pressure is about 7000 psi and the desired temperature is about 1400° C., the pressure and temperature of the admixture being maintained for about 20 to 140 minutes. Thereafter the mold is allowed to cool and the ingot removed. The ingot may then be used in manufacturing a product for use in industry, such as a plunger for use in the glass making industry.

35 When an object is needed having a blind opening therein it can be manufactured from an ingot formed in a mold in which the mold includes a floating cylinder, the cylinder forming the blind opening in the completed ingot.

40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495

as from the ingot of FIG. 3, that is, a plunger useable in the glass container manufacturing industry.

#### DESCRIPTION OF THE PREFERRED EMBODIMENT

The first step in manufacturing an object having heat, thermal shock, corrosion and wear resistance is to formulate a composition. This is achieved by thoroughly admixing powder components, such as in a grinding operation and more particularly such as in a ball milling machine. The powder compositions are formed of NiAl powder admixed with at least one of CrB<sub>2</sub> powder and TiB<sub>2</sub> powder. Optionally, a small amount of Y<sub>2</sub>O<sub>3</sub> powder may be added to any of the compositions as a sintering aid to assist in compaction of the powder mixture at high temperature. A small amount of elemental nickel may also be optionally added to act as a glue to hold the different powders together.

Up to five percent of the total powder mixture may comprise elemental nickel. If higher percentages are of elemental nickel are used it softens the resulting ingot formed upon hot pressing. About three percent by weight elemental nickel is preferably used based on the weight of CrB<sub>2</sub> used. If CrB<sub>2</sub> is a component of the powder mixture, the elemental nickel is preferably premixed with the CrB<sub>2</sub> before mixing with the other powders. Whether or not CrB<sub>2</sub> is used in a powder mixture, elemental nickel is preferably added in an amount of less than five percent by weight with the range of from one to five percent by weight being preferred.

Like any of the powders used in the compositions of the present invention, the elemental nickel is preferably ball milled to a size of between one and two microns prior to mixing with other powders and hot pressing. Usually, ball milling for a period of between about 1 and 48 is sufficient to form a uniform mixture having an average particle size of between one and two microns and very little deviation in size.

In a broad sense, the present invention relates to a composition comprising: (1) at least one member selected from the group consisting of (a) and (b), wherein (a) is about 10 to about 90 percent by weight CrB<sub>2</sub> powder and (b) is about 10 to about 80 percent by weight TiB<sub>2</sub> powder; (2) up to about five percent by weight powdered elemental nickel; (3) up to about four percent by weight Y<sub>2</sub>O<sub>3</sub> powder; and (4) NiAl powder present in an amount of up to about 90 percent by weight, wherein the powders are thoroughly admixed.

One preferred powder composition according to the present invention comprises between about 20 percent by weight and about 90 percent by weight CrB<sub>2</sub> powder, up to about five percent by weight metallic or elemental nickel, up to about four percent by weight Y<sub>2</sub>O<sub>3</sub> and the balance NiAl powder. Another powder composition according to the present invention comprises up to about 60 percent by weight CrB<sub>2</sub> powder, between about 10 and about 60 percent by weight TiB<sub>2</sub> powder, up to about four percent by weight Y<sub>2</sub>O<sub>3</sub>, up to about five percent by weight elemental nickel, and the balance being NiAl powder. Yet another composition of the present invention comprises 17-80 percent by weight TiB<sub>2</sub> powder, up to four percent by weight Y<sub>2</sub>O<sub>3</sub> and the balance NiAl powder. Compositions consisting essentially of these powder mixtures and consisting only of these powder mixtures are also preferred.

When the powder compositions are used in a process according to the present invention, an ingot is formed by hot pressing. An object formed from the ingot exhib-

its excellent heat, thermal shock, corrosion and wear resistant characteristics.

The exact amount of each powder to be used in a mixture depends upon the desired hardness and application of a formed ingot. For instance, if an ingot is to be machined into a tool for use in a wire drawing process, it is preferred that the tool exhibit a Rockwell C hardness of between about 60 and 62. These tools include reducing rolls, push rolls, pulling rolls, guide spools and swaging dies. Together, these tools are used to reduce copper and other metal ingots into wire form. Steel, platinum and tungsten can also be drawn into wire form by using such tools. Not only is it important that the tools exhibit a Rockwell C hardness of between 60 and 62, but they must also be able to work metals at very high temperature. For example, copper ingots are drawn into wire form while at a temperature of about 1900° F.

To achieve the desired hardness and high temperature resistance, a composition is used comprising between 30 and 50 percent by weight CrB<sub>2</sub>, up to five percent by weight elemental nickel, up to four percent by weight Y<sub>2</sub>O<sub>3</sub> and the balance NiAl powder. It has been found that compositions containing over 50 percent by weight CrB<sub>2</sub> have too high a hardness for this application. Similar compositions having a CrB<sub>2</sub> content of between about 38 and 42 percent by weight are even more preferred for wire drawing tool applications.

Ingots made from the compositions of the present invention can also be used to make tool insert blanks having a Rockwell C hardness of between about 70 and 75. To achieve this high hardness, a composition having an even higher amount of CrB<sub>2</sub>, compared to the compositions used for wire drawing tools, is hot pressed to form an ingot. The composition for forming a tool insert blank comprises between about 60 and 80 percent by weight CrB<sub>2</sub>, up to five percent by weight elemental nickel, up to four percent by weight Y<sub>2</sub>O<sub>3</sub> and the balance NiAl powder. More preferably, the composition comprises between 68 and 74 percent by weight CrB<sub>2</sub> with an amount of about 70 percent by weight being even more preferred.

For applications where the composition is to be formed into a plunger used to form bottles from molten glass, it is desirable that a formed ingot exhibit excellent heat, thermal shock, corrosion and wear resistance. The plunger must have a high hardness and resist scratching caused by impurities in the molten glass. The plunger must also not react with molten glass.

To achieve these properties, an ingot formed from a composition according to the present invention is provided which can be machined into a plunger having a Rockwell C hardness of about 70. The composition preferably contains between about 10 and about 40 percent by weight TiB<sub>2</sub> which enhances the heat and thermal shock resistance of a formed ingot. The composition preferably comprises up to about 80 percent by weight CrB<sub>2</sub>, between about 10 and about 40 percent by weight TiB<sub>2</sub>, up to five percent by weight elemental nickel, up to four percent by weight Y<sub>2</sub>O<sub>3</sub>, and the balance NiAl powder. More preferably, the composition comprises between about 30 and 60 percent by weight CrB<sub>2</sub>, between about 20 and about 30 percent by weight TiB<sub>2</sub>, up to five percent by weight elemental nickel, up to four percent by weight Y<sub>2</sub>O<sub>3</sub>, and the balance NiAl powder. In each of the compositions, it is preferred that at least about 10 percent by weight NiAl be included. One preferred composition comprises

about 60 percent by weight  $\text{CrB}_2$ , about 10 percent by weight  $\text{TiB}_2$ , about one percent by weight elemental nickel, up to four percent by weight  $\text{Y}_2\text{O}_3$ , and the balance NiAl powder.

Any of the compositions used for the applications discussed above may be reinforced with ceramic particulates, fibers or whiskers. Preferred ceramic particulates, fibers or whiskers which are used as reinforcing structures include ceramics such as  $\text{TiB}_2$ ,  $\text{Al}_2\text{O}_3$ ,  $\text{B}_4\text{C}$ ,  $\text{TiC}$  and  $\text{SiC}$ . If used, the reinforcing ceramic particles, whiskers or fibers are preferably added in an amount of up to about 50 percent by weight based on the total weight of the powder composition. For tool blank inserts, compositions reinforced with  $\text{SiC}$  whiskers are particularly preferred.

In one test of the composition a mixture of 55.3% nickel aluminide (NiAl) powder, 42.7% titanium diboride ( $\text{TiB}_2$ ) powder and 2% by total weight of yttria oxide ( $\text{Y}_2\text{O}_3$ ) powder was ball milled 12 hours in a zirconia grinding media. Ball milling was used for mixing the powders and reducing particle size. The powder mixture was then separated from the grinding media by using sieves and a shaker. An ingot was obtained by pouring a measured amount of powder into a graphite mold assembly for hot, high temperature pressing.

The ingot was manufactured utilizing the processes shown in FIGS. 1-2. A tubular die body 10 has a central opening 12 therethrough. The die body is preferably formed of a conductive graphite material. Received within a first end 14 of the die body is a plug cylinder 16 which may be made of carbon or low conductive graphite.

Received in the second end 18 of the die body 10 is a tubular piston member 20 having a central opening 22 therein. The tubular piston member 20 is, like the plug cylinder 16, preferably formed of carbon or low conductive graphite.

Telescopically received within central opening 22 in the tubular piston member 20 is a floating cylinder 24 that may be formed of carbon or low conductive graphite.

The powder composition 26, as previously described, is placed within the die body central opening 12 between plug cylinder 16 and tubular piston member 20. The floating cylinder 24 is positioned at its selected depth within the powder.

Surrounding the die body 10 is an inductive coil 28 that preferably is formed of tubular copper to permit the circulation of cooling fluid therethrough as indicated by the arrows 30. An alternating current voltage source is applied at 32 to heat the die body and the powder composition 26 by induction.

Pressure is applied to the powder 26 by rams 34 and 36 although, of course, one of these can be stationary. High pressure is required on powder 26 during the fusion process and in the preferred arrangement, the pressure is applied at about 7000 psi. At the same time, AC energy is applied to the inductive coil 28 to heat the powder 26 to a temperature of about 1400 degrees C. This pressure at this temperature is maintained for about 20 to 140 minutes to fuse the powder into a solidified ingot.

After the pressure and heating steps, die body 10 is allowed to cool and the ingot removed. The ingot 38 of FIG. 3 has an opening 40 therein conforming to the portion of floating cylinder 24 extending beyond the end of the tubular piston member 20 during the manufacturing process.

The process of FIGS. 1 and 2 is shown more or less diagrammatically. The die body is preferably continually surrounded by an inert gas during the manufacturing processes and the use of carbon felts and alumina furnace boards can be employed to enclose the die body and the other components during the pressure and heating stages of the manufacturing process.

The ingot 38 of FIG. 3 can be used to manufacture a finished product by machining the ingot into the desired configuration. FIG. 4 illustrates a plunger 42 useable in the glass container manufacturing industry of the type that can be made out of ingot 38. The external shape of ingot 38 can be varied according to the configuration of the die body plug cylinder 16 and the tubular piston member 20 and floating piston 24 employed in the ingot manufacturing process. The configuration of opening 40 can be varied according to the shape of floating cylinder 24.

#### EXAMPLE I

A series of test specimens were made by the process described above except the following. A mixture (hereinafter referred to as #1 mix) was made of 490 grams of HCST Corp Amperit 290.3 NiAl powder 69-31, spec. -45 + 5.6, was ball milled with 10 grams of yttrium oxide ( $\text{Y}_2\text{O}_3$ ) powder grade 5600, 99.99%, from MOLYCORP, INC. for 24 hours. Then a 10% titanium diboride sample was made by adding 10 grams  $\text{TiB}_2$ , made by UNION CARBIDE grade HCT-F, to 90 grams of #1 mix plus 0.20 gram  $\text{Y}_2\text{O}_3$ . This mixture was then ball milled for 12 hours. A similar process was used for 20% through 90%  $\text{TiB}_2$  samples, where the 90%  $\text{TiB}_2$  had 1.8 grams of  $\text{Y}_2\text{O}_3$ .

The material properties are shown in Table I. Sample preparation was accomplished by standard metallurgical polishing procedures. Hardness was measured with a Wilson Tucan Microhardness instrument with a 10 kilogram load and a Vickers diamond pyramid indenter, 136° angle. The filar readings were made at 200 $\times$  and converted to Rockwell "C" scale by chart.

Shown in Table I, the specimens were harder with increasing % of titanium diboride up to 80%, after which it decreases. The sudden drop in hardness at 90%  $\text{TiB}_2$  was the result of insufficient matrix to hold the  $\text{TiB}_2$  together. Extensive amount of porosity was observed at the 90 and 100% loads. The 100%  $\text{TiB}_2$  can be made significantly harder by hot pressing at much higher temperatures and pressures.

#### EXAMPLE II

Test specimens were made and processed as described in Example I, except that titanium diboride was kept at 40% and  $\text{Y}_2\text{O}_3$  was varied by 1%, 1.3%, 2%, 3.39%, 4.7% and 6.7%. The rate of increase in hardness was maximum at approximately 2% of  $\text{Y}_2\text{O}_3$ .

TABLE I

| % #1 Mix* | % OF $\text{TiB}_2$ | HARDNESS R"C" |
|-----------|---------------------|---------------|
| 100       | 0                   | 30-34.0       |
| 85        | 15                  | 52.7          |
| 83        | 17                  | 59.8          |
| 75        | 25                  | 61.7          |
| 60        | 40                  | 66.0          |
| 50        | 50                  | 68.0          |
| 40        | 60                  | 69.3          |
| 30        | 70                  | 70.6          |
| 20        | 80                  | 71.0          |
| 10        | 90                  | 53.0          |

TABLE I-continued

| % #1 Mix* | % OF TiB <sub>2</sub> | HARDNESS R"C" |
|-----------|-----------------------|---------------|
| 0         | 100                   | 54.0          |

Table I was compiled from 4 test runs with hot pressing times varying from 30 to 60 minutes at 7000  $\pm$  200 psi and temperature at 1400  $\pm$  10°.

\*#1 mix = 98% NiAl + 2% Y<sub>2</sub>O<sub>3</sub> by weight

NiAl = 69.2% Ni + 30.8% Al

TABLE II

| % #1 MIX* | % OF TiB <sub>2</sub> | HARDNESS R"C" |
|-----------|-----------------------|---------------|
| 90        | 10                    | 59.2          |
| 50        | 50                    | 70.5          |
| 40        | 60                    | 73.5          |

|    |    |      |
|----|----|------|
| 30 | 70 | 74.5 |
| 20 | 80 | 48.6 |
| 10 | 90 | 54.9 |

Table II was compiled from 1 test run with hot pressing time at 45 minutes at 7000 psi and temperature at 1400  $\pm$  10°.

\*#1 mix = 98% NiAl + 2% Y<sub>2</sub>O<sub>3</sub> by weight

NiAl = 69.2% Ni + 30.8% Al

The addition of CrB<sub>2</sub> to the mixture of TiB<sub>2</sub>, Y<sub>2</sub>O<sub>3</sub> and NiAl significantly enhances the hardness of a formed ingot. Depending on the desired application and hardness of an ingot formed from the powder mixture, the amount of CrB<sub>2</sub> added to the first admixture may vary as discussed above. The present invention contemplates the use of CrB<sub>2</sub> added in an amount of up to 80 percent by weight.

Compositions comprising a 1:1:1 ratio of CrB<sub>2</sub>, TiB<sub>2</sub> and NiAl and a small amount of Y<sub>2</sub>O<sub>3</sub> and/or elemental nickel have provided ingots having Rockwell C hardness measurements of greater than 70, as shown below in Table IV. High hardness values and other desirable properties are also exhibited by ingots made from compositions of the present invention comprising 25 percent by weight TiB<sub>2</sub>, 35 percent by weight CrB<sub>2</sub>, 33 percent by weight NiAl, two percent by weight Y<sub>2</sub>O<sub>3</sub>, and five percent by weight elemental nickel.

Table III below shows the data obtained during a hot press run of various compositions. Example 4 in the table shows the results of experiments done on compositions comprising 41 percent by weight NiAl powder, 29.4 percent by weight TiB<sub>2</sub> and 29.4 percent CrB<sub>2</sub> powder. The results indicate that ingots formed from the composition of Example 4 can be used to form objects which have excellent properties for molten glass plunger applications.

Table III shows the time, temperature, relative percentage of kilowatts (KW), the pressure exerted on the composition (Psig), the displacement of a ram measured in inches, and a dial indicator reading used to determine when the ram has almost stopped moving or other notes.

The temperature readings in Table III are taken from a thermal couple disposed three inches deep in the wall

of the die jacket. To determine the pounds per square inch that the sample powder is subjected to, the measured Psig is multiplied by the area of the ram in square inches (12.56) divided by the area of the inside of the die jacket (1.44 square inches). Thus, a sample subjected to 720 Psig is subjected to 6280 Psi.

After the samples are hot pressed into an ingot, they are removed from the die and sand-blasted to be cleaned. The cleaned ingot is then polished on a LECO unit, for example, model #VP-150 Vari-Pol by Leco Corp., St. Joseph, Mich. Samples are then tested for hardness and grain boundary appearance to estimate fracture toughness.

TABLE III

| Ex. No. | Mixture                                                        | Time     | Temp (C.) | % KW  | Psig    | Displacement  | Notes    |
|---------|----------------------------------------------------------------|----------|-----------|-------|---------|---------------|----------|
| III     | 50% CrB <sub>2</sub><br>50% NiAl                               | 10 mins. | 1300-1359 | 60-40 | 480-600 | 9 5/16-9 3/16 | 4361 psi |
| IV      | 29.4% TiB <sub>2</sub><br>29.4% CrB <sub>2</sub><br>41% NiAl   | 29 mins. | 1415-1432 | 40-40 | 650-700 | 9 1/2-9       |          |
| V       | 33.3% TiB <sub>2</sub><br>33.3% CrB <sub>2</sub><br>33.3% NiAl | 50 mins. | 1440-1480 | 40-30 | 820-825 | 9 1/2-9 1/4   |          |
| VI      | 33.3% TiB <sub>2</sub><br>33.3% CrB <sub>2</sub><br>33.3% NiAl | 50 mins. | 1448-1455 | 30-33 | 825-815 | 9 1/4-9 1/2   |          |

Hardness is tested to determine (1) a Filar reading from a TUKON® microhardness tester (available from Wilson® Instruments, Binghamton, N.Y.), (2) a 136° diamond pyramid hardness number, and (3) the Rockwell hardness number. Table IV below, shows the hardness measurements of numerous samples. It is clear that the 50:50 mixture of CrB<sub>2</sub> and NiAl can be hot pressed into an ingot having excellent hardness.

TABLE IV

| Ex. No. | Mixture                                                        | Filar Reading | 136° Diamond Pyramid Hardness # | Rockwell Hardness # |
|---------|----------------------------------------------------------------|---------------|---------------------------------|---------------------|
| III     | 50% CrB <sub>2</sub><br>50% NiAl                               | 251           | 1175                            | 71.5                |
| IV      | 29.4% TiB <sub>2</sub><br>29.4% CrB <sub>2</sub><br>41% NiAl   | 214           | 1610                            | 76.7                |
| V       | 33.3% TiB <sub>2</sub><br>33.3% CrB <sub>2</sub><br>33.3% NiAl | 248           | 1205                            | 71.5                |
| VI      | 33.3% TiB <sub>2</sub><br>33.3% CrB <sub>2</sub><br>33.3% NiAl | 254           | 1150                            | 70.8                |

In the preparation of the compositions according to the present invention, various organic binders and/or pelletizing agents may be used as grinding aids or for pelletizing. Pelletizing primarily changes the powder from dust to a material that can be poured into die cavities. Binders and pelletizers which may be used include methanol, starch, corn starch, methylcellulose (e.g. Methocel, available from Dow Chemical, Midland, Mich.,) polyvinyl alcohol, numerous fatty acids. One of the more preferred binders is polyvinyl alcohol (PVA). The organic binders burn-off at or before a temperature of 365° C. is reached, leaving no ash or an insignificant amount of an ash residue.

If alcohol is used for a pelletizing agent, the amount of alcohol which may be used is up to about 25 percent by weight based on the total weight of the powder composition.

The above examples illustrate that the mixtures of powders according to the present invention enable the formation of an ingot which be used to form an object having excellent heat, thermal shock, corrosion and wear resistance.

The claims and the specification described the invention presented and the terms that are employed in the claims draw their meaning from the use of such terms in the specification. The same terms employed in the prior art may be broader in meaning than specifically employed herein. Whenever there is a question between the broader definition of such terms used in the prior art and the more specific use of the terms herein, the more specific meaning is meant.

While the invention has been described with a certain degree of particularity, it is manifest that many changes may be made in the details of construction and the arrangement of components without departing from the spirit and scope of this disclosure. It is understood that the invention is not limited to the embodiments set forth herein for purposes of exemplification, but is to be limited only by the scope of the attached claim or claims, including the full range of equivalency to which each element thereof is entitled.

What is claimed is:

1. A method of manufacturing an ingot for use in making an object having heat, thermal shock, corrosion and wear resistant characteristics comprising: combining about 17-80%  $Ti_1B_2$  powder, about 0.0-4.0%  $Y_2O_3$  powder and the balance of NiAl powder to form a mixture; milling the mixture for about 10 to 48 hours to form a finely admixed composition; placing the composition in a mold; subjecting the composition in the mold to high pressure and temperature for a time to cause the composition to fuse into a high hardness ingot; and cooling the ingot and removing it from the mold.

2. The method of manufacturing an ingot according to claim 1 wherein said composition in said mold is subjected to a pressure of about 7000 psi and a temperature of about 1400° C.

3. The method of manufacturing an ingot according to claim 2 in which such heat and pressure is applied for about 20 to 140 minutes.

4. The method of manufacturing an ingot according to claim 1 wherein said mold is encompassed in an inert atmosphere during the application of heat and pressure.

5. The method of manufacturing an ingot according to claim 1 wherein the mold in which said composition is placed is formed at least in part by a tubular die body of conductive graphite and wherein high temperature is applied to said composition by an inductance coil surrounding said tubular die body.

6. The method of manufacturing an ingot according to claim 5 wherein the mold in which said composition is placed is formed in part by said tubular die body having opposed open ends, a cylindrical plug member extending within one said end of tubular die body, a tubular piston member extending telescopically within the other said end of said tubular die body and a floating cylinder member telescopically received in said tubular piston member, said composition being received within said tubular die body between said plug member and said piston members, said floating cylinder member extending beyond tubular piston member into the composition, the ingot being formed in part around said floating cylinder member.

7. A composition comprising: about 17-80%  $TiB_2$  powder, about 0.0-4.0%  $Y_2O_3$  powder, and the balance NiAl powder, the powders being thoroughly admixed by ball milling for a period of about 10 to 48 hours.

8. A composition according to claim 7 including the addition of a ceramic reinforcing components selected from the group comprising,  $TiB_2$ ,  $Al_2O_3$ ,  $B_4C$ ,  $TiC$ , and  $SiC$  and mixtures thereof, such reinforcing component being in the form of platelets, particulate, fibers or whiskers.

9. A powder composition comprising: at least one member selected from the group consisting of (a) and (b), wherein (a) is about 10 to about 90 percent by weight  $CrB_2$  powder and (b) is about 10 to about 80 percent by weight  $TiB_2$  powder; up to about five percent by weight powdered elemental nickel; up to about four percent by weight  $Y_2O_3$  powder; and NiAl powder present in an amount of up to about 90 percent by weight, wherein said powders are thoroughly admixed.

10. The composition according to claim 9, comprising between about 10 and about 80 percent by weight  $CrB_2$  powder, and between about 10 and 40 percent by weight  $TiB_2$  powder.

11. The composition as in claim 9, comprising between about 30 and about 60 percent by weight  $CrB_2$  powder and between about 20 and 30 percent  $TiB_2$  powder.

12. The composition according to claim 9, comprising between about 20 and about 90 percent by weight  $CrB_2$  powder, up to five percent by weight elemental nickel, up to four percent by weight  $Y_2O_3$  powder and the balance NiAl powder.

13. The composition according to claim 12, comprising between about 60 and 80 percent by weight  $CrB_2$  powder.

14. The composition according to claim 9, comprising between about 30 and about 50 percent by weight  $CrB_2$  powder, up to five percent by weight elemental nickel, up to four percent by weight  $Y_2O_3$  powder and between about 41 and 70 percent by weight NiAl powder.

15. A composition comprising according to claim 11, further comprising reinforcing ceramic particles, whiskers or fibers selected from the group consisting of  $TiB_2$ ,  $Al_2O_3$ ,  $B_4C$ ,  $TiC$  and  $SiC$ , said reinforcing ceramic particles, whiskers or fibers being added in an amount of up to about 50 percent by weight based on the total weight of the powder composition.

16. A composition according to claim 9, comprising elemental nickel present in an amount of up to about 5.0 percent by weight.

17. The composition according to claim 11, wherein said powders are thoroughly admixed by ball milling for a period of between about 10 to 48 hours.

18. A method of manufacturing an ingot for use in making an object having heat, thermal shock, corrosion and wear resistant characteristics, said method comprising the steps of:

combining at least one member selected from the group consisting of (a) and (b), wherein (a) is about 10 to about 90 percent by weight  $CrB_2$  powder and (b) is about 10 to about 80 percent by weight  $TiB_2$  powder, with up to about five percent by weight powdered elemental nickel, with up to about four percent by weight  $Y_2O_3$  powder, and with NiAl

**11**

powder in an amount of up to about 90 percent by weight, to form a powder mixture; milling the powder mixture for about 1 to 48 hours to form a finely admixed composition; placing the composition in a mold; subjecting the composition in the mold to high pressure and temperature for a time to cause the composition to fuse into a high hardness ingot; and cooling the ingot and removing it from the mold.

19. A method according to claim 18, further comprising the step of mixing said finely admixed composition with an organic binder or pelletizing agent prior to placing the composition in the mold.

20. A method according to claim 18, wherein said step of combining comprises combining between about 15

**12**

10 and about 80 percent by weight  $\text{CrB}_2$  powder with about 10 to about 40 percent by weight  $\text{TiB}_2$  powder and with  $\text{NiAl}$  powder present in an amount of up to about 80 percent by weight to form a mixture.

5 21. A method according to claim 18, wherein said step of combining comprises combining about 60 and 80 percent by weight  $\text{CrB}_2$  powder with about up to about five percent by weight powdered elemental nickel, with up to about four percent by weight  $\text{Y}_2\text{O}_3$  powder, and the balance  $\text{NiAl}$  powder to form a powder mixture.

10 22. An ingot made by the process according to claim 18.

\* \* \* \* \*

20

25

30

35

40

45

50

55

60

65